

## UNITED STATES PATENT OFFICE

2,116,274

## ALUMINIUM ALLOY

Yonosuke Matuenaga, Naka-ku, Yokohama,  
JapanNo Drawing. Original application May 8, 1936,  
Serial No. 78,723. Divided and this application  
November 12, 1936, Serial No. 110,553.  
In Japan May 13, 1935

## 1 Claim. (Cl. 75—146)

This application is a divisional from applicant's copending application Serial No. 78,723, filed May 8, 1936.

This invention relates to an aluminium alloy containing main and auxiliary elements, the main elements consisting of 2 to 5% magnesium, 6 to 14% zinc, 0.2 to 2.0% nickel, 0.01 to 1.5% iron, 0.1 to 1.0% silicon and the rest substantially aluminium keeping the condition that the content of silicon is always greater than that of iron, while the auxiliary elements consisting of a metal selected from the group of 0.1 to 1.5% manganese, a few percentage of cobalt, molybdenum, vanadium, tungsten, titanium, lithium and beryllium. The object of the invention is to obtain an aluminium alloy which has a great tensile strength and great elongation especially when subjected under heat treatment.

Example of the alloy showing percentages of the elements employed and also tensile strength and elongation when the alloys are subjected under a mode of tempering and annealing is given as follows:

| Example                               | I%   | II%  |
|---------------------------------------|------|------|
| Mg                                    | 2.5  | 2.5  |
| Zn                                    | 9.0  | 9.0  |
| Ni                                    | 0.5  | 1.0  |
| Fe                                    | 0.2  | 0.2  |
| Si                                    | 0.6  | 0.6  |
| Mn                                    | 0.8  | 0.8  |
| Al                                    | Rest | Rest |
| Tensile strength kg./cm. <sup>2</sup> | 58.5 | 60.3 |
| Elongation %                          | 15   | 12   |

It is acknowledged from repeated experiments that addition of a few percentage of cobalt, molybdenum, vanadium, tungsten, titanium, lithium or beryllium does not appreciably modify the properties of the alloy so that alloys containing one or more of the above elements are considered equivalent alloys to each other. 5

As to be seen from the above example, the new alloy has a very great tensile strength and a very great elongation which are hardly obtainable in known aluminium alloys. 10

As to mutual action of the elements of the new alloy, it is supposed as follows. A part of magnesium may combine with silicon to form magnesium silicide, and another part of magnesium may be alloyed with a part of zinc and a part of aluminium to form various three elemental alloys of different percentage. Further nickel may be alloyed with iron. These chemical compounds and alloys may crystal out in the main element, viz., aluminium and may be uniformly distributed therein. Further, when manganese is employed, this manganese not only acts as reducing agent, but also hinders the growth of particles of zinc-manganese-aluminium alloys and also of nickel-iron alloy so that the distribution of the alloy may be promoted. 15 20 25

What I claim is:—

An aluminium alloy containing 2 to 5% magnesium, 6 to 14% zinc, 0.2 to 2% nickel, 0.01 to 1.5% iron, 1 to 1% silicon, the silicon content being always greater than the iron content, 1 to 1.5% manganese and the rest aluminium. 30

YONOSUKE MATUENAGA.

35